

## UNITED STATES PATENT OFFICE.

JOHN F. WANDERSEE, OF HIGHLAND PARK, AND JOHN L. McCLOUD, OF DEARBORN, MICHIGAN, ASSIGNORS TO FORD MOTOR COMPANY, OF DETROIT, MICHIGAN, A CORPORATION OF DELAWARE.

## ALLOY.

No Drawing.

Application filed July 19, 1923. Serial No. 652,609.

*To all whom it may concern:*

Be it known that we, JOHN F. WANDERSEE and JOHN L. McCLOUD, citizens of the United States, residing, respectively, at 5 Highland Park and Dearborn, in the county of Wayne and State of Michigan, have invented new and useful Improvements in Alloys, of which the following is a specification.

10 The object of our invention is to provide an alloy of relatively slight cost which will have heat resisting qualities in a large degree.

15 A further object of our invention is to provide an alloy which is especially adapted to retain its structure and more especially its surface structure although subjected to repeated rapid changes of temperature from atmospheric temperature to many hundred 20 degrees.

25 A further object of our invention is to provide an alloy which is readily formed and which will fulfill the requirements for the valves for heavy duty, internal combustion engines.

With these and other objects in view our invention consists in the arrangement, construction and combination of the various 30 elements and formulas of our invention as described in the specification and claimed in the claims.

In the practice of our invention we have found that we can combine relatively small quantities of chromium and silicon with a 35 low carbon steel to thereby form a valve alloy which has proven very satisfactory for use in a large number of tractor engines which are run continuously with a full load so that the valves used were subjected to the 40 hardest possible type of test. We are aware that it has already been proposed to combine chromium and silicon with steel to form a heat resisting alloy for valves but we have found that the alloys so proposed were very 45 expensive on account of the large amounts, relatively, of silicon and chromium which were introduced into the alloy and on account of the difficulty of properly admixing such a large proportion of these elements. 50 Our experiments have shown that with the formula hereafter given we have produced an alloy which has a structural and surface

suitability which is as far as we can determine fully equal to any alloy of the large number which we have tried in connection 55 with our experiments and yet at the same time it is very much cheaper than the special alloys which are designed for resisting temperature variations and high temperatures.

Analysis of our alloy shows the following 60 proportions: carbon, .25% to .45%; manganese, .25% to .40%; chromium, 1.85% to 2.50%; silicon, 3.60% to 4.20%; phosphorus, .03% to .10%; sulphur, .04% to .10%.

This formula represents an average from 65 a large number of analyses taken from a large number of different heats of our alloy and should be, therefore, considered representative. If the quantities of chromium or silicon are materially increased above the 70 amounts here specified, we have found that some proportions reduce the efficiency of the metal to resist heat and that other proportions do not materially increase the efficiency of the metal to resist heat. Variations in the carbon content of considerable 75 amounts do not affect the heat resisting qualities of this metal and the same is substantially true in connection with the manganese content. If, however, the quantity 80 of phosphorus is increased above .300 of 1% or of sulphur above .400 of 1% the quality becomes noticeably poorer. If the silicon and chromium contents are reduced more than 1% under those amounts given in this 85 formula, then a decrease in the resistance of the metal to the action of heating becomes very noticeable.

The principal advantage of our improved alloy rests in the fact that we are able to 90 produce a material which is thoroughly adapted to use in valves for internal combustion engines which are subjected to high temperatures and that this alloy can be produced at a cost very materially less than that 95 of any other alloy with the same heat resisting qualities that we have been able to discover.

Some changes may be made in the proportions of the ingredients of our improved 100 alloy and various methods may be used for securing the desired analysis. The use of this alloy is of course not limited to the valves but of course may be extended to any

application where a metal is desired which will retain its structure and surface under continued high temperatures and which also will withstand rapid variations of temperature of many hundred degrees.

We claim as our invention:

- 5 1. An alloy with high heat resisting qualities having ferrous base combined with carbon from .25% to .45%; manganese, .25% to .45%; chromium, 1.85% to 2.50%; and silicon, 3.60% to 4.20%.
- 10 2. An alloy with high heat resisting qualities having a ferrous base combined with carbon .25% to .45%; manganese, .25% to .45%; chromium, 1.85% to 2.50%; and silicon, 3.60 to 4.20%; and, neither more than
- 15

.03% of phosphorus nor over .04% of sulphur.

3. An alloy with high heat resisting qualities comprising ferrous base combined with 20 carbon from .25% to .45%; manganese, .25% to .45%; chromium 1.85% to 2.50%; and silicon, 3.60% to 4.20%, and not more than .50% of impurities.

4. A heat resisting alloy having a low carbon ferrous base combined with from .85% to 25 3.50% of chromium and from 2.60% to 5.20% of silicon.

Dated July 5, 1923.

JOHN F. WANDERSEE.  
JOHN L. McCLOUD.